# EUROPEAN PATENT SPECIFICATION

(11) **EP 4 118 308 B1**
(45) Date of publication and mention of the grant of the patent: **01.05.2024**
(21) Application number: 20710909.1
(22) Date of filing: 11.03.2020
(51) Int. Cl.: F01L 1/32, F01L 3/04

(54) **METHOD OF CONFIGURING A GAS EXCHANGE VALVE ASSEMBLY IN AN INTERNAL COMBUSTION PISTON ENGINE AND A GAS EXCHANGE VALVE**
VERFAHREN ZUR KONFIGURATION EINER GASWECHSELVENTILANORDNUNG IN EINEM HUBKOLBENMOTOR UND GASWECHSELVENTIL
PROCÉDÉ DE CONFIGURATION D'UN ENSEMBLE SOUPAPE D'ÉCHANGE DE GAZ DANS UN MOTEUR À PISTON À COMBUSTION INTERNE ET SOUPAPE D'ÉCHANGE DE GAZ

(43) Date of publication of application: 18.01.2023
(73) Proprietor: Wärtsilä Finland Oy, 65100 Vaasa (FI)
(72) Inventor: SÖCHTING, Sven, 65100 Varkaus (FI); SUUTALA, Jyrki, 65100 Vaasa (FI)
(74) Representative: Genip Oy
(86) International application number: PCT/EP2020/056517
(87) International publication number: WO 2021/180315

(56) References cited:
- EP-A2- 0 126 323
- WO-A1-98/19084
- DE-A1- 4 111 381
- DE-A1-102004 063 941
- US-B2- 10 364 844

## Description

### Technical field

The present invention relates to method of configuring a gas exchange valve assembly in an internal combustion piston engine according to claim 1.

The present invention relates to gas exchange valve of an internal combustion piston engine, comprising a valve stem and a valve disc at a first end of the stem, wherein the valve disc has a sealing surface.

### Background art

The interface of the combustion engine valve sealing surface and its seat surface are sensitive to non-conformity of the surfaces e.g. due to misalignment and shape deformation either during assembly or via distortions resulting from temperature and pressure during engine operation. The nonconformity of the surfaces may lead to insufficient sealing properties and or wear due to increased contact stress, both resulting in failure of the component requiring pre-mature engine shut down and repair. In particular the effects resulting from engine operation are difficult to predict and compensate.

EP0126323 A2 discloses a component for a combustion chamber of a high speed diesel engine, of the type having sliding surfaces provided with wear-protection layers which are used up during the running-in period, and to a process for obtaining such layers. The publication recognizes that for the purpose of extending the life of diesel engines and the maintenance intervals thereof it is sought to encourage a correct running-in by means of the application of wear-protection layers on the sliding surfaces of the mechanical elements forming components of the engine, and in particular those forming the combustion chamber. There is disclosed a component of a combustion chamber of a diesel engine in particular, of the type comprising at least one sliding surface coated with a wear-protection layer which can be worn away during a running-in period, said wear layer is constituted by a nitride based heat diffusion layer containing a percentage by weight of nitrogen lying between about 4% and 12%. The process for forming a wear-protection layer over a sliding surface of an element forming a component of a combustion chamber of a diesel engine, which can be worn away during the running-in period of the said engine. The layer comprises a phase of gaseous nitriding of the said surface performed with ammonia or nitrogen ionised at a temperature less than or equal to 600°C in conditions such as to obtain on the said surface the formation of a layer of nitrides substantially of 6 - type. Even if EP0126323 generally refers to a number components provided with wear-protection layers for a combustion chamber of a diesel engine, and while the component may be also a valve seat, the enabling disclosure of the document relates to piston rings of the engine.

GB983120 A discloses a surface coating on periphery of piston rings which accelerates the wear rate until the rings are bedded-in. The piston rings according to the document having their peripheral faces covered with a bonding agent, an abrasive and a lubricant. The proposed coating is not suitable for the temperatures and contact pressures in gas exchange valve they are surface smoothing but would not remove a sufficient amount of material to create the dimensional change required.

Publication US7225781 B2 discloses particularly an engine valve used for opening or closing intake and exhaust paths of an automobile or a motorcycle engine. The document teaches a method for surface treating an engine valve made from titanium or titanium alloy in order to form a hardened coating having improved abrasion and impact resistances. A hardened layer is formed on the surface of the engine valve by furnishing the surface of the engine valve with oxygen as a solid solution and then forming a coating on the surface of the hardened layer with a PVD process.

Document DE 102004063941 A1 discloses a valve rotating device for exhaust valves, especially of ships' diesel engines, is supported in a valve housing between a lower and an upper drive element for the valve spindle. The rotation of the valve spindle is effected through a rotary cylinder with engages with a stationary support cylinder. The rotary cylinder and stationary support cylinder interengage via a helical gearing, whereby the rotary cylinder is connected to the valve spindle via an overrunning device and the support cylinder is fastened on the valve housing side.

Document DE 102004063941 A1 discloses piston rings and/or a piston in an internal combustion engine of the diesel type, particularly a two-stroke crosshead engine. In a newly manufactured state radial outer surface of the piston rings and/or a section of the radial outer surface of the piston is/are provided with a running-in layer comprising a solid-state lubricant and a metallic binder, and the running-in layer has a thickness of at least 0.1 mm in the radial direction and is made of a material which, stated in percentage by weight and apart from commonly occurring impurities, includes from 5 to 60% of solid-state lubricant, such as graphite, and 40 to 95% of the metallic binder, such as Ni, Al, Si, and optionally up to 15% of an organic binder, and that the macro-hardness of the running-in layer is less than 300 He30.

An object of the invention is to provide method of configuring a gas exchange valve assembly in an internal combustion piston engine by means of which the valve disk and the valve seat of the valve assembly are made in conformity with each other during the engine is running.

An object of the invention is to provide a gas exchange valve by means of which the valve disk and the valve seat of the valve assembly are made in conformity with each other during the engine is running.

### Disclosure of the Invention

Objects of the invention can be met substantially as is disclosed in the independent claims and in the other claims describing more details of different embodiments of the invention.

A method of configuring a gas exchange valve assembly in an internal combustion piston engine comprises:
- providing a gas exchange valve
- providing a valve seat
- arranging an abrasive wearing overlay on a base material at a region of a sealing surface of first one of the gas exchange valve disk and the valve seat,
- assembling the valve seat into a gas exchange valve body
- assembling the valve into the gas exchange valve body
and while running the engine, rotating the valve around its longitudinal axis during its lift and/or close movements such that the sealing surface of the valve detach and/or touch the valve seat in the gas exchange valve body by a movement comprising a rotational component, wherein the abrasive wearing overlay machines the sealing surface of second one of the valve disk and the valve seat into conformity with each other.

This provides an in-situ machining that improves the conformance of valve and valve seat sealing surfaces for engine operation conditions.

According to an embodiment of the invention rotational position of the valve is changed by rotating it in one direction such that the abrasive overlay makes dimensional changes to sealing surface of the second one of the valve disk and the valve seat until the abrasive overlay is worn off from the sealing surface.

According to an embodiment of the invention the method comprises arranging an abrasive wearing overlay on the base material at a region of a sealing surface of the gas exchange valve disk and while running the engine, the valve is rotated around its longitudinal axis during its lift and/or close movements such that the sealing surface of the valve detach and/or touch the valve seat in the gas exchange valve body by a movement comprising a rotational component, wherein the abrasive wearing overlay machines the sealing surface of second one of the valve seat into conformity with the sealing surface of the valve until the abrasive surface has lost its abrasive effect. The abrasive effect is lost when the abrasive overlay has worn off or the abrasive particles have been dislodged from the overlay.

The abrasive wearing overlay containing abrasive material on the valve sealing surface machines the respective the seat surface to achieve conformance of the surfaces during running of the engine. This is achieved by making dimensional changes in the seat surface i.e. in addition to removing any local micro-protrusion on the valve seat surface use of the valve according to the invention makes the valve seat sealing surface to conform with the form of the valve disk through positive dimensional changes which changes a median line of a real surface of the valve disk. The overlay comprises abrasive particles of nano scale to micro scale. The abrasive particles will dislodge from the sealing surface during the machining process and will be mainly removed along the exhaust gases and engine lubrication oil.

The abrasive effect can be controlled by controlling the thickness of the coating and/or size of the abrasive particle. Due to the abrasive machining the abrasives are detached from the sealing surface, however the coating may be designed to further assist or improve the contact surface friction and wear performance. This technique will improve conformance of the contact surfaces and in the progress reducing maximum contact pressure and wear off the valve and valve seat surface and minimizes adhesive contact in the sealing surface during early stage of the engine running process.

According to an embodiment of the invention the abrasive wearing overlay is configured to wear away from the surface within less than 200 running hours of the engine.

According to an embodiment of the invention arranging an abrasive wearing overlay on a sealing surface comprises arranging a matrix substance and abrasive particles embedded to the matrix substance on the base material.

According to an embodiment of the invention arranging an abrasive wearing overlay on a sealing surface comprises arranging a metal matrix with carbide particles therein as abrasives on the base material.

A gas exchange valve of an internal combustion piston engine, comprising a valve stem and a valve disc at a first end of the stem, wherein the valve disc has a sealing surface where a base material of valve disc sealing surface is provided with an abrasive wearing overlay.

According to an embodiment of the invention the base material comprises a hardened layer at its outer surface and the hardened layer is provided with the abrasive wearing overlay on top of it.

According to an embodiment of the invention the abrasive wearing overlay consist of a matrix substance and abrasive particles embedded to the matrix substance.

According to an embodiment of the invention the abrasive wearing overlay consist of metal matrix with carbide particles therein as abrasives.

According to an embodiment of the invention carbide is tungsten carbide.

According to an embodiment of the invention the carbide grain size is 0.5 -20 µm.

According to an embodiment of the invention the abrasive wearing overlay comprises a first abrasive overlay and a second abrasive overlay, wherein the first abrasive overlay has a first amount of abrasive particles and the second abrasive overlay has a second amount of abrasive particles.

According to an embodiment of the invention the abrasive wearing overlay comprises a first abrasive overlay and a second abrasive overlay, wherein the first abrasive overlay has abrasive particles of first grain size and the second abrasive overlay has abrasive particles of second grain size.

According to an embodiment of the invention the abrasive wearing overlay comprises a diamond-like carbon (DLC) coating having a thickness more than 45 µm.

The overlay may be multi layered e.g. having different sizes of the abrasive particles in each layer.

Generally the base material selected for use in the gas exchange valve, particularly the valve disk is considerably hard material minimizing the wear. Depending on the base material and the abrasive overlay it might be desirable to provide an additional treatment to the base material for improving the attachment of the abrasive overlay.

The abrasive overlay can be obtained on the base material making use of following methods, being not exclusive list but currently considered as advantageous methods.

### Physical vapor deposition (PVD)

Physical vapor deposition (PVD) describes a variety of vacuum deposition methods which can be used to produce thin films and coatings. PVD is characterized by a process in which the material goes from a condensed phase to a vapor phase and then back to a thin film condensed phase. The most common PVD processes are sputtering and evaporation. PVD is used in the manufacture of items which require thin films for mechanical, optical, chemical or electronic functions. Some examples of implementing PVD method are as follows.

Cathodic Arc Deposition, in which a high-power electric arc discharged at the source material blasts away some into highly ionized vapor to be deposited onto the workpiece.

Electron beam physical vapor deposition, in which the material to be deposited is heated to a high vapor pressure by electron bombardment in high vacuum and is transported by diffusion to be deposited by condensation on the cooler workpiece.

Evaporative deposition in which the material to be deposited is heated to a high vapor pressure by electrical resistance heating in high vacuum.

Close-space sublimation, where the material and substrate are placed close to one another and radiatively heated.

Pulsed laser deposition, in which a high-power laser ablates material from the target into a vapor.

Sputter deposition, in which a glow plasma discharge bombards the material sputtering some away as a vapor for subsequent deposition.

Pulsed electron deposition, whereas highly energetic pulsed electron beam ablates material from the target generating a plasma stream under nonequilibrium conditions.

According to an embodiment the abrasive wearing layer comprises nanometer and/or micro-meter sized diamonds embedded in PVD coating.

### Diamond-like carbon coating using PVD coating

Diamond-like carbon (DLC) is a class of amorphous carbon material that displays some of the typical properties of diamond. DLC is usually applied as coatings to other materials that could benefit from some of those properties. The various forms of DLC can be applied to almost any material that is compatible with a vacuum environment.

Even if DLC coatings are generally applied as a wear or corrosion protection coating, it has been discovered that if the coating is applied to form an increased thickness it exhibits a reverse behavior and becomes abrasive to an extent applicable to the invention. Suitable thickness to obtain the effect required to implement the invention is 45 micrometers or more.

According to an embodiment the abrasive wearing layer comprises nanometer and/or micro-meter sized diamonds embedded in DLC coating.

According to an embodiment the abrasive wearing layer comprises nanometer and/or micro-meter sized diamonds embedded in coating provided by a combination of Cold spray coating and DLC coating.

### Cold spray of tungsten carbide composite coating

A cold spray coating technology is a coating deposition method. Solid powders are accelerated in a supersonic gas jet to velocities up to ca. 1200 m/s. During impact with the substrate, particles undergo plastic deformation and adhere to the surface. The kinetic energy of the particles, supplied by the expansion of the gas, is converted to plastic deformation energy during bonding..

The abrasive overlay comprises a metallic matrix into which carbides are embedded forming the abrasive part of the overlay. Metallic matrix is arranged to have a hardness of 200 - 350 HV and the carbides hardness is around 1000-2000HV. Metallic matrix suitable for use in connection with the valve seat overlay according to the invention is NiCrBSi-alloy or CU based alloy. Carbide may be e.g. Tungsten Carbide, WC. The carbide grain size is between 0.5 - 20 micrometers. The carbides will initially be fully embedded in the coating and as the metal matrix starts wearing carbides will be protruding and act as abrasives. Also, a friction enhancing materials may be added to the matrix

According to an embodiment the abrasive wearing layer comprises nanometer and/or micro-meter sized diamonds embedded in cold spray coating.

### Smart Coating

A graded coating or sometimes referred to as a smart coating is applicable in connection with the present invention. It is technically a monolayer coating but its composition changes gradual over its thickness. Smart coating can be obtained by using e.g. thermal and cold spray techniques. The smart coating can be tailored to needs at a certain time in the life of the coating by adding different abrasive and matrix compositions to the coating during the process. There can be different sizes of abrasives, different mixture grades of the metal matrix or additional material to improve thermal properties e.g. copper or even solid lubricants to improve tribological properties of the abrasive wearing overlay.

It is possible to obtain several advantageous effects. Firstly it is possible to improve running in and conformance of engine valves and valve seat surfaces. Secondly it is possible to reduce maximum contact pressure and wear off the valve/valve seat surface due to better conformance of the sealing surfaces and also minimize adhesive contact during early stage of the running in process. The abrasive particles will disappear during the engine is used.

The abrasive wearing overlay can be multi layered e.g. having different sizes of the abrasive particles in each layer.

The base material of both components, namely valve disc and valve seat, are extremely stiff, such that they will not conform elastically to each other, therefore the abrasive method is needed to embed the surfaces with each other.

The exemplary embodiments of the invention presented in this patent application are not to be interpreted to pose limitations to the applicability of the appended claims. The verb "to comprise" is used in this patent application as an open limitation that does not exclude the existence of also unrecited features. The features recited in depending claims are mutually freely combinable unless otherwise explicitly stated. The novel features which are considered as characteristic of the invention are set forth in particular in the appended claims.

### 3D printing

3D printing method or a so called hybrid approach where a 3D printed overlay is created on top of a metallic matrix can be utilized with success. The 3D printed metals generally show a rough, and therefore abrasive surface, however using 3D printing similar material approach to the spray coating could be used.

### Brief Description of Drawings

In the following, the invention will be described with reference to the accompanying exemplary, schematic drawings, in which
Figure 1 depicts schematically valve assembly in which the sealing sur-face of the valve is provided with an abrasive overlay,
Figure 2 depicts schematically a valve assembly in which the sealing surface of the valve seat is provided with an abrasive overlay,
Figure 3 depicts schematically a structure of the sealing surface provided with an abrasive overlay according to an embodiment of the invention, and
Figure 4 depicts schematically a structure of the sealing surface provided with an abrasive overlay according to another embodiment of the invention.

### Detailed Description of Drawings

Figure 1 depicts schematically gas exchange valve assembly 10 of an internal combustion piston engine arranged to a cylinder head 12 of the engine. The gas exchange valve assembly is configured to controllably admit entry of combustion air into a combustion chamber 14 of the engine and removal of exhaust gases from the combustion chamber 14. The gas exchange valve assembly comprises a gas exchange valve 16, which may called simply as a valve, and a valve seat 18. The valve seat 18 is a ring-like member which has a sealing surface against which an intake or an exhaust valve rests during the stage of the engine operating cycle when that valve is closed. The sealing surface prevents gas leaking from the combustion chamber to the intake air receiver and to the exhaust gas manifold and it also functions as heat transfer surface for releasing heat from the valve 16 to the cylinder head 12. The valve 16 comprises a valve stem 16.1 and a valve disk 16.2 and a first end of the stem 16.1. The valve is supported by a valve guide 22 in the cylinder head.

The valve assembly is also provided with a valve rotator 20 which is configured to rotate the valve around its longitudinal axis A by positive action, while the valve is moved in the direction of the longitudinal axis A. The valve seat 18 is coaxial with the valve 16. The valve rotator may be of a type know as such for a skilled person in the art, for example a so called ball spring rotator, or such as is disclosed e.g. in the publication EP0768450 B1 or DE102013013229 A1.

A so-called "rotocap" valve rotator incorporates a ball-retaining plate with ramped circumferential grooves for balls to roll along. A small spring pushes each of these balls to one side. A Belleville-type dished spring washer fits over these balls to form an upper race, which is supported on its outer edge by a spring-seat retainer. This retainer holds the whole assembly together and also provides a seat for the helical-coil valve springs. In the closed position of the valve, the dished spring washer is suspended between the spring-seat retainer and the ball-retainer, so that the balls move freely to a first end of the ramp and abut against the end of the groove. During opening stage of the valve, the dished spring washer deflects with the increase in the compression load on the valve spring. The outer edge of the dished washer bears against the spring-seat retainer as before, but the inner part of the washer now bears against the balls and hence pushes them along their ramps. The ramps are so shaped that, as contact with the washer is maintained, the spring-seat retainer is rotated and hence the valve is rotated by the same amount. As the valve closes, the washer comes back to its original position between the spring-seat retainer and the ball-retainer. This releases the load on the balls due to which the small bias springs now push the balls up their ramps and thereby bring the spring-seat retainer and the valve assembly back to its starting position.

The valve disc is provided with a sealing surface 24 at its radial periphery region, which surface is typically at an angle with respect to the longitudinal axis A of the valve. Respectively, the valve seat 18 is provided with a sealing surface 26 which is ideally parallel to and in conformity with the sealing surface 24 of the valve. The valve disk 16.2 is made of a hard base alloy material, which is durable against wear. An abrasive wearing overlay 28 is arranged over the base material at the region of at least the sealing surface 24 of the valve 16. The sealing surface of the valve 16 may comprise a hardened layer which is provided with the abrasive wearing overlay 28. The valve 16 is made of material which experiences minimal deformations during its lifespan and is machined accurately to intended dimensions.

In the figure 1 the valve 16 is at a position where it has just started its lift i.e. opening movement the sealing surface 24 of the valve has detached from the sealing surface 26 of the valve seat 18. The area of the sealing surfaces is shown in more detailed in the enlarged view encircled in the figure. In the view A there is indicated a cut-out line II-II which refer to the figure 2, in which the valve seat 18 is shown along the cut-out II-II. The view A depicts exemplary an angular flaw or non-conformance 30 in the seat surface 26. As is depicted in figure 2 the non-conformance may be a local, non-symmetrical deviation from a circular shape at a plane in the direction of the longitudinal axis A. Of course, the present invention is applicable regardless of the shape of the non-conformance. The gas exchange valve assembly in an internal combustion piston engine is configured for use such that firstly a gas exchange valve 16 and a valve seat 18 are provided and an abrasive wearing overlay is arranged on a base material at a region of a sealing surface of first one of the gas exchange valve disk and the valve seat. In particularly referring to the figure 1 the abrasive wearing overlay is arranged on the sealing surface of the gas exchange valve disk 16.2. The abrasive wearing overlay is arranged to cover the area of the valve 16 which is intended to form its sealing surface. In this case the dimensional accuracy of the valve disk is important because the valve seat is accommodated according to the shape of the valve disk.

Next, the valve seat 18 and the valve 16 are assembled into a gas exchange valve body. While running the engine, the valve 16 is rotated around its longitudinal axis during its lifting and/or closing movements such that the sealing surface 24 of the valve detach and/or touch the sealing surface 26 valve seat 18 in the gas exchange valve body by a movement comprising a rotational component. Thus when the abrasive wearing overlay simultaneously moves axially and angularly in respect to the longitudinal axis, it also machines the sealing surface of second one of the valve disk and the valve seat into conformity with each other by forming a rotational fit between the surfaces. In particularly referring to the figure 1 the abrasive wearing overlay arranged on the sealing surface of the gas exchange valve disk 16.2 machines the sealing surface 26 of the valve seat 18 into conformity with the sealing surface 24 of the valve disk 16.2. The rotational position of the valve 16 is changed by rotating it in one direction. The abrasive overlay makes dimensional changes to sealing surface until the abrasive overlay or the abrasive material in the overlay is worn off from the sealing surface.

Figure 3 depicts schematically a valve assembly in which the sealing surface of the valve seat is provided with an abrasive overlay 28. This embodiment is applicable when the valve seat is made of material which experiences minimal deformations during its lifespan and is machined accurately to intended dimensions.

Figure 4 depicts schematically a structure of the base material 40, 41 provided with an abrasive overlay 28 according to an embodiment of the invention. The base material comprises a substrate i.e. the material of the base material of the valve disk 16.1 (or alternative the valve seat 18) which may have its outer surface area 41 hardened. The outer surface are 41 is a so called working surface which comes to use when the abrasive overlay has been worn out. The outer surface 41 can be hardened making use of methods know as such, like a heat treatments, shot peening. A thick (advantageously 1-3mm) hard intermediate coating can be applied between the base material and the abrasive coating. The intermediate coating can be manufactured via Plasma Transferred Arc method or laser cladding. The intermediate coating material can be stellite or similar.

Figure 5 depicts schematically a structure of the base material 40, 41 provided with an abrasive overlay 28', 28" according to another embodiment of the invention. The abrasive wearing overlay 28', 28" has different abrasive properties at its top region 28" and bottom region 28'. Like in the embodiment of the figure 4 the base material comprises a substrate i.e. the material of the base material of the valve disk 16.1 (or alternative the valve seat 18) which may have its outer surface area 41 hardened. The outer surface are 41 is a so called working surface which comes to use when the abrasive wearing overlay has been worn out. The abrasive wearing overlay 28', 28" may optionally comprise distinct layers having different abrasive properties. The abrasive wearing overlay 28', 28" may also comprise regions from bottom to top having gradually changing abrasive properties. The different abrasive properties may be accomplished be providing different particle, or grain size of the abrasive particles and/or different amount of particles in the overlay.

The abrasive wearing overlay comprises a first abrasive overlay 28' and a second abrasive overlay 28" on top of the first abrasive overlay, wherein the first abrasive overlay 28' has abrasive particles of first grain size and the second abrasive overlay 28" has abrasive particles of second grain size, greater than the first grain size.

The abrasive wearing overlay comprises a first abrasive overlay 28' and a second abrasive overlay 28", wherein the first abrasive overlay 28' has a fist amount, i.e. concentration of abrasive particles and the second abrasive overlay 28" has a second amount i.e. concentration of abrasive particles, being more than the first amount of abrasive particles.

As an example of the method according to the invention the abrasive wearing overlays may be formed as follows: The base material can be any suitable hard material selected in a view of minimizing wear and deformations in the use but also ensuring adequate corrosion resistance. Suitable materials are such as martensitic stainless steel, silicon-chromium steels, austenitic chromium-nickel steels or nickel-based super alloys. The base material may be hardened making use of suitable methods, such as heat treatment, shot peening, surface rolling etc. The following table shows some applicable selections for abrasive overlays in the method of the present invention.

| **Selection** | **First abrasive overlay (28 / 28')** | **Second abrasive overlay (28")** |
|---|---|---|
| 1 | - Cold spray coating of NiCrBSi-alloy or CU based alloy | - |
| | -metal matrix, hardness of 200 - 350 HV | |
| | -abrasives containing carbides having hardness of 1000-2000HV | |
| | - carbide, diameter 0.5 -20 µm | |
| 2 | - Diamond-like carbon (DLC) coating, thickness of the coating more than 45 µm | - |
| 3 | - PDV coating method, metallic material | - PDV coating method, metallic material |
| | - abrasives of tungsten carbide, diameter is 0.5 -20 µm | - abrasives of tungsten carbide, diameter is 0.5 -20 µm |
| 4 | - PDV coating method | - |
| | - abrasives of tungsten carbide, diameter is 0.5 -20 µm | |
| 5 | - Smart coating | Optional smart coating |
| | - Coating method any one of the 1 to 4, having gradually changing abrasive concentration and/or diameter | - Coating method any one of the 1 to 4, having gradually changing abrasives, abrasive concentration, and/or abrasive geometry e.g. diameter |

While the invention has been described herein by way of examples in connection with what are, at present, considered to be the most preferred embodiments, it is to be understood that the invention is not limited to the disclosed embodiments, but is intended to cover various combinations or modifications of its features, and several other applications included within the scope of the invention, as defined in the appended claims. The details mentioned in connection with any embodiment above may be used in connection with another embodiment when such combination is technically feasible.

## Claims

1. A method of configuring a gas exchange valve assembly (10) in an internal combustion piston engine comprising:
- providing a gas exchange valve (16)
- providing a valve seat (18),
- arranging an abrasive wearing overlay (28) on a base material at a region of a sealing surface (24) of first one of the gas exchange valve disk (16.2) and the valve seat (18),
- assembling the valve seat (18) into a gas exchange valve body
- assembling the valve into the gas exchange valve body
- and while running the engine, rotating the valve (16) around its longitudinal axis during its lift and/or close movements such that the sealing surface (24) of the valve detach and/or touch the valve seat (18) in the gas exchange valve body by a movement comprising a rotational component, wherein the abrasive wearing overlay (28) machines the sealing surface (24) of second one of the valve disk (16.2) and the valve seat (18) into conformity with each other.

2. A method of configuring a gas exchange valve in an internal combustion piston engine according to claim 1, **wherein** the rotational position of the valve is changed by rotating it in one direction such that the abrasive overlay (28) makes dimensional changes to sealing surface (24) of the second one of the valve disk (16.2) and the valve seat (18) until the abrasive overlay (28) is worn off from the sealing surface (24).

3. A method of configuring a gas exchange valve in an internal combustion piston engine according to claim 1, **wherein** the method comprises arranging an abrasive wearing overlay (28) on the base material at a region of a sealing surface (24) of the gas exchange valve disk (16.2) and while running the engine, the valve is rotated around its longitudinal axis during its lift and/or close movements such that the sealing surface (24) of the valve detach and/or touch the valve seat (18) in the gas exchange valve body by a movement comprising a rotational component, wherein the abrasive wearing overlay (28) machines the sealing surface (24) of second one of the valve seat (18) into conformity with the sealing surface (24) of the valve, until the abrasive surface has lost its abrasive effect.

4. A method of configuring a gas exchange valve in an internal combustion piston engine according to claim 1, **wherein** the abrasive wearing overlay (28) is configured to wear away from the surface within less than 200 running hours of the engine.

5. A method of configuring a gas exchange valve in an internal combustion piston engine according to claim 1, **wherein** arranging an abrasive wearing overlay (28) on a sealing surface (24) comprises arranging a matrix substance and abrasive particles embedded to the matrix substance on the base material.

6. A method of configuring a gas exchange valve in an internal combustion piston engine according to claim 1, **wherein** arranging an abrasive wearing overlay (28) on a sealing surface (24) comprises arranging a metal matrix with carbide particles therein as abrasives on the base material.

7. A gas exchange valve of an internal combustion piston engine, comprising a valve stem and a valve disc at a first end of the stem, wherein the valve disc has a sealing surface (24), **characterized in that** a base material of valve disc sealing surface (24) is provided with an abrasive wearing overlay (28).

8. A gas exchange valve according to claim 7, **characterized in that** abrasive wearing overlay (28) is configured to wear away from the surface within less than 200 running hours of the engine.

9. A gas exchange valve according to claim 7, **characterized in that** the base material comprises a hardened layer at its outer surface and the hardened layer is provided with the abrasive wearing overlay (28) on top of it.

10. A gas exchange valve according to claim 7 or 9, **characterized in that** the abrasive wearing overlay (28) consist of a matrix substance and abrasive particles embedded to the matrix substance.

11. A gas exchange valve according to claim 10, **characterized in that** the abrasive wearing overlay (28) consist of metal matrix with carbide particles therein as abrasives.

12. A gas exchange valve according to claim 11, **characterized in that** carbide is tungsten carbide.

13. A gas exchange valve according to claim 11, **characterized in that** the carbide grain size is 0.5 -20 µm.

14. A gas exchange valve according to claim 7, **characterized in that** the abrasive wearing overlay (28) comprises a first abrasive overlay (28') and a second abrasive overlay (28"), wherein the first abrasive overlay (28') has a first amount of abrasive particles and the second abrasive overlay (28") has a second amount of abrasive particles.

15. A gas exchange valve according to claim 7, **characterized in that** the abrasive wearing overlay (28) comprises a first abrasive overlay (28') and a second abrasive overlay (28"), wherein the first abrasive overlay (28') has abrasive particles of first grain size and the second abrasive overlay (28") has abrasive particles of second grain size.

16. A gas exchange valve according to claim 7, **characterized in that** the abrasive wearing overlay (28) comprises a diamond-like carbon (DLC) coating having a thickness more than 45 µm.

## Patentansprüche

1. Verfahren zum Konfigurieren einer Gaswechselventilanordnung (10) in einem Hubkolbenmotor, umfassend:
- Bereitstellen eines Gaswechselventils (16)
- Bereitstellen eines Ventilsitzes (18)
- Einrichten einer abrasiven Verschleißdeckschicht (28) auf einem Basismaterial in einem Bereich einer Dichtfläche (24) eines ersten des Gaswechselventiltellers (16.2) und des Ventilsitzes (18),
- Einbauen des Ventilsitzes (18) in einen Gaswechselventilkörper
- Einbauen des Ventils in den Gaswechselventilkörper
- und während des Betriebs der Maschine, Drehen des Ventils (16) um seine Längsachse während seiner Hub- und/oder Schließbewegung derart, dass sich die Dichtfläche (24) des Ventils von dem Ventilsitz (18) in dem Gaswechselventilkörper durch eine Bewegung, die eine Drehkomponente umfasst, löst und/oder diesen berührt, wobei die abrasiven Verschleißdeckschicht (28) die Dichtfläche (24) des zweiten des Ventiltellers (16.2) und des Ventilsitzes (18) in Übereinstimmung miteinander bearbeitet.

2. Verfahren zum Konfigurieren eines Gaswechselventils in einem Hubkolbenmotor nach Anspruch 1, wobei die Drehposition des Ventils durch sein Drehen in einer Richtung geändert wird, so dass die abrasive Deckschicht (28) dimensionale Änderungen an der Dichtfläche (24) des zweiten des Ventiltellers (16.2) und des Ventilsitzes (18) macht, bis die abrasive Deckschicht (28) von der Dichtfläche (24) abgenutzt ist.

3. Verfahren zum Konfigurieren eines Gaswechselventils in einem Hubkolbenmotor nach Anspruch 1, wobei das Verfahren das Einrichten einer abrasiven Verschleißdeckschicht (28) auf dem Basismaterial in einem Bereich einer Dichtfläche (24) des Gaswechselventiltellers (16.2) umfasst, und während des Betriebs des Motors das Ventil um seine Längsachse während seiner Hub- und/oder Schließbewegung derart gedreht wird, dass die Dichtfläche (24) des Ventils in dem Gaswechselventilkörper durch eine Bewegung, die eine Drehkomponente umfasst, gelöst wird und/oder diesen berührt, wobei die abrasive Verschleißdeckschicht (28) die Dichtfläche (24) des zweiten des Ventilsitzes (18) in Übereinstimmung mit der Dichtfläche (24) des Ventils bearbeitet, bis die abrasive Oberfläche ihre abrasive Wirkung verloren hat.

4. Verfahren zum Konfigurieren eines Gaswechselventils in einem Hubkolbenmotor nach Anspruch 1, wobei die abrasive Verschleißdeckschicht (28) dazu konfiguriert ist, von der Oberfläche innerhalb von weniger als 200 Betriebsstunden des Motors abgenutzt zu werden.

5. Verfahren zum Konfigurieren eines Gaswechselventils in einem Hubkolbenmotor nach Anspruch 1, wobei das Einrichten einer abrasiven Verschleißdeckschicht (28) auf einer Dichtfläche (24) das Einrichten einer Matrixsubstanz und abrasiver Teilchen, die in der Matrixsubstanz eingebettet sind, auf dem Basismaterial umfasst.

6. Verfahren zum Konfigurieren eines Gaswechselventils in einem Hubkolbenmotor nach Anspruch 1, wobei das Einrichten einer abrasiven Verschleißdeckschicht (28) auf einer Dichtfläche (24) das Einrichten einer Metallmatrix mit Carbidteilchen darin als Schleifmittel auf dem Basismaterial umfasst.

7. Gaswechselventil eines Hubkolbenmotors, das einen Ventilschaft und einen Ventilteller an einem ersten Ende des Schafts umfasst, wobei der Ventilteller eine Dichtfläche (24) aufweist, **dadurch gekennzeichnet, dass** ein Basismaterial der Ventiltellerdichtfläche (24) mit einer abrasiven Verschleißdeckschicht (28) versehen ist.

8. Gaswechselventil nach Anspruch 7, **dadurch gekennzeichnet, dass** die abrasive Verschleißdeckschicht (28) konfiguriert ist, um von der Fläche innerhalb von weniger als 200 Betriebsstunden des Motors abgenutzt zu werden.

9. Gaswechselventil nach Anspruch 7, **dadurch gekennzeichnet, dass** das Basismaterial eine gehärtete Schicht an seiner Außenfläche umfasst und die gehärtete Schicht mit der abrasiven Verschleißdeckschicht (28) an ihrer Oberseite versehen ist.

10. Gaswechselventil nach Anspruch 7 oder 9, **dadurch gekennzeichnet, dass** die abrasive Verschleißdeckschicht (28) aus einer Matrixsubstanz und abrasiven Teilchen, die in der Matrixsubstanz eingebettet sind, besteht.

11. Gaswechselventil nach Anspruch 10, **dadurch gekennzeichnet, dass** die abrasive Verschleißdeckschicht (28) aus Metallmatrix mit Carbidteilchen als Schleifmittel darin besteht.

12. Gaswechselventil nach Anspruch 11, **dadurch gekennzeichnet, dass** das Carbid Wolframcarbid ist.

13. Gaswechselventil nach Anspruch 11, **dadurch gekennzeichnet, dass** die Carbidkorngröße 0,5 - 20 µm beträgt.

14. Gaswechselventil nach Anspruch 7, **dadurch gekennzeichnet, dass** die abrasive Verschleißdeckschicht (28) eine erste abrasive Deckschicht (28') und eine zweite abrasive Deckschicht (28'') umfasst, wobei die erste abrasive Deckschicht (28') eine erste Menge an abrasiven Teilchen aufweist, und die zweite abrasive Deckschicht (28'') eine zweite Menge an abrasiven Teilchen aufweist.

15. Gaswechselventil nach Anspruch 7, **dadurch gekennzeichnet, dass** die abrasive Verschleißdeckschicht (28) eine erste abrasive Deckschicht (28') und eine zweite abrasive Deckschicht (28'') umfasst, wobei die erste abrasive Deckschicht (28') abrasive Teilchen in einer ersten Korngröße aufweist, und die zweite abrasive Deckschicht (28'') abrasive Teilchen in einer zweiten Korngröße aufweist.

16. Gaswechselventil nach Anspruch 7, **dadurch gekennzeichnet, dass** die abrasive Verschleißdeckschicht (28) eine diamantähnliche Carbonbeschichtung (DLC-Beschichtung), die eine Dicke von mehr als 45 µm aufweist, umfasst.

## Revendications

1. Procédé de configuration d'un ensemble de soupape d'échange de gaz (10) dans un moteur à piston à combustion interne comprenant de :
- fournir une soupape d'échange de gaz (16),
- prévoir un siège de soupape (18),
- disposer un revêtement d'usure abrasif (28) sur un matériau de base au niveau d'une région d'une surface d'étanchéité (24) du premier parmi le disque de soupape d'échange de gaz (16.2) et le siège de soupape (18),
- assembler le siège de soupape (18) dans un corps de soupape d'échange de gaz,
- assembler la soupape dans le corps de la soupape d'échange de gaz,
- et pendant le fonctionnement du moteur, faire tourner la soupape (16) autour de son axe longitudinal lors de ses mouvements de levage et/ou de fermeture de telle sorte que la surface d'étanchéité (24) de la soupape détache et/ou touche le siège de soupape (18) dans le corps de soupape d'échange de gaz par un mouvement comprenant une composante de rotation, dans lequel le revêtement d'usure abrasif (28) usine la surface d'étanchéité (24) du deuxième du disque de soupape (16.2) et du siège de soupape (18) en conformité l'un avec l'autre.

2. Procédé de configuration d'une soupape d'échange de gaz dans un moteur à piston à combustion interne selon la revendication 1, dans lequel la position de rotation de la soupape est modifiée en la faisant tourner dans une direction de telle sorte que le revêtement abrasif (28) apporte des modifications dimensionnelles à la surface d'étanchéité (24) du deuxième du disque de soupape (16.2) et du siège de soupape (18) jusqu'à ce que le revêtement abrasif (28) soit usé de la surface d'étanchéité (24).

3. Procédé de configuration d'une soupape d'échange de gaz dans un moteur à piston à combustion interne selon la revendication 1, dans lequel le procédé comprend la disposition d'un revêtement d'usure abrasif (28) sur le matériau de base au niveau d'une région d'une surface d'étanchéité (24) du disque de soupape d'échange de gaz (16.2) et pendant le fonctionnement du moteur, la soupape tourne autour de son axe longitudinal pendant ses mouvements de levage et/ou de fermeture de telle sorte que la surface d'étanchéité (24) de la soupape se détache et/ou touche le siège de soupape (18) dans le corps de soupape d'échange de gaz par un mouvement comprenant une composante de rotation, dans lequel le revêtement d'usure abrasif (28) usine la surface d'étanchéité (24) du deuxième siège de soupape (18) en conformité avec la surface d'étanchéité (24) de la soupape, jusqu'à ce que la surface abrasive ait perdu son effet abrasif.

4. Procédé de configuration d'une soupape d'échange de gaz dans un moteur à piston à combustion interne selon la revendication 1, dans lequel le revêtement d'usure abrasif (28) est configuré pour s'user de la surface en moins de 200 heures de fonctionnement du moteur.

5. Procédé de configuration d'une soupape d'échange de gaz dans un moteur à piston à combustion interne selon la revendication 1, dans lequel la disposition d'une couche d'usure abrasive (28) sur une surface d'étanchéité (24) comprend la disposition d'une substance matricielle et de particules abrasives incorporées à la substance matricielle sur le matériau de base.

6. Procédé de configuration d'une soupape d'échange de gaz dans un moteur à piston à combustion interne selon la revendication 1, dans lequel la disposition d'un revêtement d'usure abrasif (28) sur une surface d'étanchéité (24) comprend la disposition d'une matrice métallique contenant des particules de carbure comme abrasifs sur le matériau de base.

7. Soupape d'échange de gaz d'un moteur à piston à combustion interne, comprenant une tige de soupape et un disque de soupape à une première extrémité de la tige, dans laquelle le disque de soupape présente une surface d'étanchéité (24), **caractérisée en ce qu'**un matériau de base de la surface d'étanchéité du disque de soupape (24) est dotée d'un revêtement d'usure abrasif (28).

8. Soupape d'échange de gaz selon la revendication 7, **caractérisée en ce que** le revêtement d'usure abrasif (28) est configuré pour s'user de la surface en moins de 200 heures de fonctionnement du moteur.

9. Soupape d'échange de gaz selon la revendication 7, **caractérisée en ce que** le matériau de base comprend une couche durcie au niveau de sa surface extérieure et la couche durcie est munie du revêtement d'usure abrasif (28) au-dessus d'elle.

10. Soupape d'échange de gaz selon la revendication 7 ou 9, **caractérisée en ce que** le revêtement d'usure abrasif (28) est constitué d'une substance matricielle et de particules abrasives incrustées dans la substance matricielle.

11. Soupape d'échange de gaz selon la revendication 10, **caractérisée en ce que** le revêtement d'usure abrasif (28) est constitué d'une matrice métallique contenant des particules de carbure servant d'abrasifs.

12. Soupape d'échange de gaz selon la revendication 11, **caractérisée en ce que** le carbure est du carbure de tungstène.

13. Soupape d'échange de gaz selon la revendication 11, **caractérisée en ce que** la taille des grains de carbure est de 0,5 à 20 µm.

14. Soupape d'échange de gaz selon la revendication 7, **caractérisée en ce que** le revêtement d'usure abrasif (28) comprend un premier revêtement abrasif (28') et un deuxième revêtement abrasif (28"), dans lequel le premier revêtement abrasif (28') comporte une première quantité de particules abrasives et le deuxième revêtement abrasif (28") comporte une deuxième quantité de particules abrasives.

15. Soupape d'échange de gaz selon la revendication 7, **caractérisée en ce que** le revêtement d'usure abrasif (28) comprend un premier revêtement abrasif (28') et un deuxième revêtement abrasif (28"), dans lequel le premier le revêtement abrasif (28') comporte des particules abrasives d'une première granulométrie et le deuxième revêtement abrasif (28") comporte des particules abrasives d'une deuxième granulométrie.

16. Soupape d'échange de gaz selon la revendication 7, **caractérisée en ce que** le revêtement d'usure abrasif (28) comprend un revêtement en carbone de type diamant (DLC) ayant une épaisseur supérieure à 45 µm.
